

## UNITED STATES PATENT OFFICE

2,069,470

PROCESS OF FINISHING SURFACES IN  
SIMULATION OF NAPPED CLOTHGuido Ariotti, Stamford, Conn., assignor to  
Atlas Powder Company, Wilmington, Del., a  
corporation of DelawareNo Drawing. Application June 1, 1933,  
Serial No. 673,929

## 1 Claim. (Cl. 91—68)

This invention relates to a new method of finishing, wherein metal, wood or composition surfaces are coated in such manner that they appear to be covered with a finely napped cloth.

- 5 My invention is particularly adapted to the finishing of small or irregular objects which can be covered with cloth only with great difficulty and at a relatively high cost. My process is equally well adapted for finishing large surfaces such as 10 burial caskets, the interior of automobile bodies and even the walls of a room. Other articles which have been successfully finished according to my process are cast iron toys, vanity cases, clock cases, lip stick holders, handbag frames 15 and radio cabinets. My process is particularly adapted for finishing relatively rough surfaces such as castings and the like as I can obtain a smooth finish of excellent appearance without the necessity of first filling and sanding, which operations are frequently necessary when enamel, 20 paint or lacquer are employed as the finishing mediums.

In carrying out my process I first apply to the surface a coating of adhesive of a nature herein- 5 after set forth. While the surface is still wet or tacky I apply cotton rayon, silk, mohair, or other suitable flock. The flock may be applied by first sprinkling a quantity on the wet surface and then shaking or vibrating the coated article 10 in such manner as to thoroughly embed the flock in the wet surface of the lacquer or other finishing material used. However, the preferred method of applying the flock is by blowing it on by means of compressed air by use of a specially 15 constructed "spray gun". When this method is employed there is no necessity of vibrating the coated object to embed the flock as the velocity 20 of the compressed air may be so regulated that the flock impinges on the wet surface with sufficient force to become thoroughly embedded 25 therein.

The cotton rayon, silk or mohair flock may be 30 previously dyed to any desired color. After the coating has become thoroughly dry or set the excess flock may be readily removed by brushing or may be blown off by means of compressed air. The finished surface will now have the general 35 appearance of having been covered with felt, duveteen or similar fabrics.

40 Under some conditions it is advantageous to use an adhesive, or other base coat, which has been pigmented to approximately match the color of the flock. This is particularly desirable where the original color of the article differs considerably 45 from that of the flock to be applied. When

transparent varnishes or lacquers are used the original color of the article may show through to such an extent as to throw the flock off shade so that the desired color is not obtained. The necessary pigment may be incorporated into the adhesive material by any of the well known methods.

The adhesive material may be applied by brushing, dipping or spraying. The spraying method is preferred, due to the fact that a large object can 10 be quickly coated and the flock deposited thereon before any portion of the surface may have become sufficiently dry to prevent the flock from adhering.

Where it is desired to apply my finish to large 15 surfaces, such as burial caskets, interior of automobile bodies and the like, it is necessary to use a slow drying finish adhesive such as a synthetic resin solution. By using a slower drying finish than lacquer it is possible to coat the entire 20 surface and then apply the flock and avoid the possibility that part of the surface may have become so dry that the flock will not adhere. I find synthetic resin solutions particularly satisfactory as they dry sufficiently slowly to allow 25 time for the flocking operation yet do not dry so slowly that production is held up. Synthetic products of the character indicated will air dry sufficiently to allow packing and shipping within two to six hours whereas paint, varnish and similar 30 materials will require eight to twenty-four hours. Synthetic resin finish may also be baked at temperatures around 200-250° F. and thoroughly dried in  $\frac{1}{2}$  to  $1\frac{1}{2}$  hours. The formula of a satisfactory pigmented synthetic resin solution 35 is shown below:

|                                         | Percent |
|-----------------------------------------|---------|
| Polyhydric alcohol-polybasic acid resin | 30      |
| Pigment                                 | 18      |
| Cobalt naphthenate                      | .1 40   |
| Mineral spirits                         | 11.9    |
| Turpentine                              | 20.0    |
| Xylol                                   | 20.0    |

A typical formula for the polyhydric alcohol-polybasic resin described above would be as follows:

|                         | Percent |
|-------------------------|---------|
| Glycerol                | 23      |
| Phthalic anhydride      | 46      |
| Linseed oil fatty acids | 31 50   |

It will be evident from these examples that practically any type of finishing material can be used as long as its drying time may be regulated to allow the application of the flock to the 55

surface while it is still sufficiently wet and tacky to secure proper adhesion. It is also desirable that the finishing material have sufficient adhesion to the surface to which it is applied in order 5 that the entire finish be sufficiently "bonded" or adherent.

The process herein described lends itself to the ornamentation of the surfaces of articles of various kinds in a highly economical but extremely 10 pleasing fashion. For example, ordinary metal buttons may be made to have every appearance of a cloth button. Toy metal furniture may be made to have the appearance of an upholstered piece of furniture. Vanity cases, pocket books, 15 and other articles too numerous to mention may be finished in all sorts of pleasing designs by coating one part of the article with a flock of one color, and then through the medium of a stencil applying a flock of a different color to produce 20 designs of many sorts. The extent of application of this method is almost limitless, and it offers marked economies in many fields of manufacture.

I do not limit myself to any particular type of adhesive finishing material so long as it is of a 25 nature to dry much faster than ordinary paints and varnishes to permit thereby of packing and shipping in much less time than would be possible where paints and varnishes are used, while

at the same time drying slow enough to permit the coating of relatively large surfaces before any part of the surface has become so dry that the flock will not adhere.

Having described my invention, what I claim 5 is:

The herein described method of finishing large surfaces such as burial caskets, interior of automobile bodies and the like, which consists of applying thereto a coating of a viscous material 10 consisting of the following ingredients:

|                                         | Percent |
|-----------------------------------------|---------|
| Polyhydric alcohol-polybasic acid resin | 30.0    |
| Pigment                                 | 18.0    |
| Cobalt naphthenate                      | 1 15    |
| Mineral spirits                         | 11.9    |
| Turpentine                              | 20.0    |
| Xylool                                  | 20.0    |

and before drying, blowing upon said viscous 20 material a body of flock corresponding substantially to the color of the said viscous material, the rate of drying of the viscous material being sufficiently slow to allow time for the application of the flock but rapid enough to air-dry sufficiently to permit packing and shipping within from two to six hours.

GUIDO ARIOTTI.